

Oct. 2, 1934.

W. A. BOUGHTON

1,975,081

FIBROUS PRODUCTS WITH INORGANIC BINDERS

Filed Sept. 12, 1932

ASBESTOS OR OTHER FIBROUS MATERIALS,  
MAY BE SATURATED WITH ADHESIVE.



Inventor

Willis A. Boughton

384

Warren G. Ogden  
her Attorney

## UNITED STATES PATENT OFFICE

1,975,081

## FIBROUS PRODUCTS WITH INORGANIC BINDERS

Willis A. Boughton, Cambridge, Mass., assignor to New England Mica Co., Waltham, Mass., a corporation of Massachusetts

Application September 12, 1932, Serial No. 632,849

15 Claims. (Cl. 154—2.6)

This invention relates to fibrous products with inorganic binders, of the class which are temperature resistant, oil resistant, and electrically insulating, and the like, of various shapes, such as 5 sheets, rings, special objects, etc., from non-combustible fibrous matter, such as asbestos, mineral wool, slag wool, and other inorganic fibrous matter, and when desired associated with mica; or such non-combustible matter may be associated 10 with combustible matter, such as cotton goods or fibres, woolen goods or fibres, paper pulp, etc., the raw material to be saturated or coated with a highly viscous adhesive aqueous association 15 of an inorganic colloid, as described hereafter, or mixtures of such viscous aqueous colloidal associations, and the combined mass suitably pressed, shaped, dried, heated, or otherwise treated mechanically. The invention also contemplates the manufacture of such products from 20 fibrous cellulose matter, or wool or the like, singly or mixed with such fibrous matter as cotton, or cotton goods, paper pulp, wool or woolen goods, etc., associated with the highly viscous adhesive aqueous colloidal association, or mixtures of such 25 colloidal associations.

An object of the invention is to provide a product which is fire resistant, oil resistant, possessing high electrical insulating properties, and which may be formed into a plurality of shapes.

30 A further object is to provide a product which may be converted into washers, gaskets, packings, etc., which remain tight and do not decompose when subjected to temperatures up to about 600° F.

35 A further object is to provide a product which in at least one stage of manufacture is reversibly thermoplastic, and which upon heating to elevated temperatures may be suitably shaped as desired, and which will become solid on cooling.

40 A further object is to effect a marked improvement in the mechanical strength of impregnated fibrous materials, especially those prepared by laying the fibres in sheet form without weaving or similar fabrication.

45 Other objects of the invention will be apparent to those skilled in the art upon reading the specification.

50 The accompanying drawing illustrates one type of fibrous product in accordance with this invention, showing a laminated sheet consisting of layers of asbestos or other fibrous material which may be impregnated with adhesive as described 55 herein, and intermediate alternate layers of ad-

hesive and flake mica, the assembled sheet thereafter baked under pressure.

In the preparation of temperature and electrical resisting and insulating materials of various kinds prepared from fibrous products, it has heretofore been difficult to secure adequate resistance to high temperatures because of the frequent necessity of using organic resins and gums as binder, and these by nature decompose at temperatures of 300–600° F., thus limiting the 60 temperatures at which the materials may be used safely in the manufacture of a large variety of products.

I have discovered that the general group of 70 inorganic substances that form highly viscous adhesive colloidal associations with water may be successfully employed in the bonding, stiffening and protecting of fibrous materials, yielding a variety of products of new and highly useful properties.

This group of colloidal inorganic binders with or without chemical modification is fully described in my several pending applications for 75 patents, as follows: Mica products with inorganic binders, filed March 9, 1931, Serial No. 521,378. General processes of bonding, filed June 22, 1931, Sr. No. 546,153. Methods of restraining crystallization, filed June 22, 1931, Sr. No. 546,154. Molded laminated mica products with inorganic 80 binders and methods of making the same (W. A. Boughton and W. R. Mansfield), filed March 18, 1932, Sr. No. 599,844.

The substances used as binders include such 85 compounds as sodium metaphosphate,  $Na_3PO_3$ ; sodium monoborate,  $NaBO_2$ ; other alkali metaphosphates and monoborates such as the respective ammonium, lithium, and potassium compounds; also a few other chemically related compounds; also a variety of salts of the element 90 beryllium; also, mixtures of these substances may be used. They are all characterized by the property of forming highly viscous adhesive aqueous colloidal associations, the viscosity usually being greater than that of glycerine and often as great as that of asphalt, or practically solid, depending on the amount of water in colloidal association with the salt molecule. These substances hold tenaciously to their colloidally attached water, as described below, yielding it up only slowly 95 at temperatures considerably above the normal boiling point of a concentrated aqueous salt solution. Definite analyses are difficult to obtain because of the abnormal physical nature of such substances, but I have found that there is still residual water associated with several of them at 100 105 110

temperatures upwards of 300° F., and in certain instances upwards of 450° F. The differences in viscosities between various concentrations of such compounds is striking. With sodium metaphosphate, for example, the 15 percent solution is less viscous than glycerine, while the 60 percent solution is as viscous as a heavy, slow-flowing tar. Solutions of ammonium metaphosphate or metaphosphoric acid may be prepared which are so viscous as to be essentially solid at ordinary temperatures. In general, the smaller amount of water associated with such an anomalous inorganic substance, the higher its viscosity at ordinary temperatures.

15 Sodium metaphosphate is known to exist in several polymeric forms. To develop in it the bonding property utilized in this invention I form an aqueous solution of the glassy hexapolymer at a temperature below the boiling point of water 20 and as rapidly as possible. The common commercial powdered sodium metaphosphate is usually a mono-, di-, or tri-polymer, and cannot be so used until after fusion when it is transformed to the glassy hexa salt. Similarly, crystalline sodium monoborate is an aqueous association, but a non-useful form in the sense of this invention. An aqueous solution if dilute shows no unusual viscosity and if concentrated crystallizes on cooling and standing, again being useless for this invention. Only when of a correct intermediate concentration, about 35 percent to about 40 percent, or higher, and heated under pressure does it become a bonding material of desirable properties. The bonding property is therefore not necessarily an inherent property but one that may be developed as the result of treatment or of careful control of conditions.

25 The fibrous matter may first be impregnated with a plastic in liquid form, such as a solution of a lacquer, then sprinkled with the aqueous inorganic colloid body, or it may be drawn through a vat containing the said aqueous inorganic colloid body, and the resulting pulp squeezed, suitably shaped and dried, or the preliminary impregnation may be omitted. The salt content in the dried product will vary with the intended use of the product, a general range of from about fifteen percent to about thirty percent of salt, by weight, on a dry basis, may be used. One dried and finished product contained 27.14 percent of sodium metaphosphate; another dried and finished product contained 23.25 percent of sodium monoborate. These products were impregnated asbestos sheets which had been rolled dry on a steam table at approximately 250° F.

(A) *Fibrous mineral products and inorganic binder*

30 The fibrous mineral products used may include asbestos in any of its several forms and preferably made up into sheet form. Also, such products as mineral wool, slag wool, etc. Thus commercial asbestos paper and asbestos cloth are very suitable materials. But in the following specification, wherever asbestos paper is specifically referred to, it must be understood that any other mineral fibre may also be employed with similar results.

35 When the inorganic binders referred to above are employed with micaceous and similar materials as described in my earlier patent applications, no observable reaction takes place between the mica and the binder. The latter under controllable conditions functions as an increasingly

viscous adhesive body, losing its associated water slowly, and yielding a product that may be molded at some definite elevated temperature depending on the temperature of the prior heating and the resulting residual colloidal water content.

40 With asbestos, however, these colloidal inorganic binders act differently. Upon saturation of the asbestos with the binder there is the expected easy absorption; and the product is then soft, flexible and capable of being shaped. But when the resulting mass or sheet is dried and heated somewhat above 220° F. it becomes inflexible, hard and semi-crystalline, due (it appears) to a chemical reaction between the binder and the complex silicate of the asbestos. Such a product in sheet form is highly useful in the manufacture of washers to withstand elevated temperatures, for the preparation of stiff, non-softening, high temperature resisting and insulating forms or special shapes, for the preparation of such forms and shapes that shall be oil resisting to a high degree, and for many other products which acquire many unique and valuable properties.

45 Moreover, when for example asbestos paper is saturated with an inorganic binder such as a viscous colloidal solution of sodium metaphosphate, and before being dried and heated is adhesively combined with a layer of integrated mica sheet prepared with inorganic binder as previously described (general process of bonding application) and the combination then pressed and heated either flat or in a mold, permanently formed products such as sheet insulation, commutator rings, and various shapes and forms may 50 be prepared that are useful in industry and an improvement over similar products made with organic binders, because of superior temperature resistance and strength at the higher temperatures.

(B) *Fibrous vegetable products and inorganic binders*

55 Inorganic binding fluids of the class described above may also be used with vegetable fibrous materials yielding a new group of valuable products having, however, the temperature limitations in use imposed by the presence of organic material. However, in the lower ranges of temperature the binder functions as a reversible 60 thermoplastic, as described above. Thus with a sheet of cellulose fibre such as paper pulp laid loosely enough to be absorbent the binder is absorbed, and the sheet may then be dried and baked best under pressures of about 200 pounds 65 per square inch at any temperature up to about 400° F.

70 Below the drying temperature the sheet is stiff and hard; but a few degrees above that temperature it is flexible and may be shaped, resuming 75 its hardness when cooled. Among the articles for which such products may be used are shoe stiffeners, clothing forms, low temperature heat and temperature resisting articles such as gaskets and the like, oil resistant members of various sorts, etc. Many other applications will be obvious to those familiar with the field of stiffened thermoplastic fibrous bodies.

I claim:

1. A bonded product containing fibrous material bonded with an aqueous colloidal association containing at least one adhesive selected from the group consisting of viscous colloidal aqueous associations of metaphosphoric acid radical com-

80

85

90

95

100

105

110

115

120

125

130

135

140

145

150

- 5 pounds, monoborates, and beryllium compounds, the dried product containing from about fifteen percent to upwards of forty percent of the compound, and bonded under pressure at temperatures upwards of 220° F., but below temperatures which will eliminate all water. 80
- 10 2. A bonded product containing inorganic material and organic material, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 85
- 15 3. A bonded product containing asbestos, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 90
- 20 4. A bonded product containing organic fibrous material, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 95
- 25 5. A bonded product containing cellulose fibrous matter, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 100
- 30 6. A molded product consisting of a shaped mass containing fibrous material, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 105
- 35 7. A molded product consisting of a shaped mass of fibrous asbestos material, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 110
- 40 8. Sheet material containing fibrous asbestos material, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 115
- 45 9. Sheet material containing fibrous asbestos associated with cellulose fibrous matter, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded at temperatures upwards of 220° F., but below temperatures which will eliminate all water. 120
- 50 10. Insulating material for commutators consisting of laminated mica and asbestos fibre, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 125
- 55 11. Composite insulating products consisting of sandwiched layers of mica and asbestos fibre, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 130
- 60 12. Composite insulating products consisting of associated mica flakes and asbestos fibre, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 135
- 65 13. Composite packing, consisting of a mass of associated mica flakes and asbestos fibre, bonded with an aqueous colloidal association containing at least one adhesive selected from the group consisting of viscous colloidal aqueous associations of metaphosphoric acid radical compounds, monoborates, and beryllium compounds, the dried product containing from about fifteen percent to upwards of forty percent of the compound, and bonded under pressure at temperatures upwards of 220° F., but below temperatures which will eliminate all water. 140
- 70 14. A bonded product containing fibrous material, said material first impregnated with an organic liquid plastic, and thereafter bonded with an aqueous colloidal association containing at least one adhesive selected from the group consisting of viscous colloidal aqueous associations of 145
- 75 8. Sheet material containing fibrous asbestos material, bonded with an aqueous colloidal association 150

metaphosphoric acid radical compounds, monoborates, and beryllium compounds, the dried product containing from about fifteen percent to about thirty percent of the compound, and bonded under pressure at a temperature of about 250° F., but below temperatures which will eliminate all water.

15. A bonded product containing vegetable fibrous material, bonded with an aqueous colloidal association containing at least one adhesive selected from the group consisting of viscous colloidal

aqueous associations of metaphosphoric acid radical compounds, monoborates, and beryllium compounds, the dried product containing from about fifteen percent to upwards of forty percent of the compound, and bonded under pressures of about 200 pounds per square inch, and at a temperature not above 400° F., but below temperatures which will eliminate all water.

80

WILLIS A. BOUGHTON. 85

14

## CERTIFICATE OF CORRECTION.

Patent No. 1,975,081.

October 2, 1934.

WILLIS A. BOUGHTON.

It is hereby certified that error appears in the printed specification of the above numbered patent requiring correction as follows: Page 3, line 82, claim 8, after "bonded" insert the words under pressure; and that the said Letters. Patent should be read with this correction therein that the same may conform to the record of the case in the Patent Office.

30 Signed and sealed this 30th day of October, A. D. 1934.

35 (Seal)

Leslie Frazer  
Acting Commissioner of Patents.

40

115

45

120

50

125

55

130

60

135

65

140

70

145

75

150

metaphosphoric acid radical compounds, monoborates, and beryllium compounds, the dried product containing from about fifteen percent to about thirty percent of the compound, and bonded under pressure at a temperature of about 250° F., but below temperatures which will eliminate all water.

15. A bonded product containing vegetable fibrous material, bonded with an aqueous colloidal association containing at least one adhesive selected from the group consisting of viscous colloidal

aqueous associations of metaphosphoric acid radical compounds, monoborates, and beryllium compounds, the dried product containing from about fifteen percent to upwards of forty percent of the compound, and bonded under pressures of about 200 pounds per square inch, and at a temperature not above 400° F., but below temperatures which will eliminate all water.

80

WILLIS A. BOUGHTON. 85

14

## CERTIFICATE OF CORRECTION.

Patent No. 1,975,081.

October 2, 1934.

WILLIS A. BOUGHTON.

It is hereby certified that error appears in the printed specification of the above numbered patent requiring correction as follows: Page 3, line 82, claim 8, after "bonded" insert the words under pressure; and that the said Letters. Patent should be read with this correction therein that the same may conform to the record of the case in the Patent Office.

30 Signed and sealed this 30th day of October, A. D. 1934.

35 (Seal)

Leslie Frazer  
Acting Commissioner of Patents.

40

115

45

120

50

125

55

130

60

135

65

140

70

145

75

150